

Aug. 15, 1939.

S. H. GRIFFITHS

2,169,797

METHOD OF CASTING SELF STRIPPING AND RAPID-COOLING STEEL INGOTS

Filed Dec. 31, 1937

2 Sheets-Sheet 1



FIG. 4.



Inventor.

Septimus H. Griffiths

By Jas. L. Skidmore,

Attorney.

Aug. 15, 1939.

S. H. GRIFFITHS

2,169,797

METHOD OF CASTING SELF STRIPPING AND RAPID-COOLING STEEL INGOTS

Filed Dec. 31, 1937

2 Sheets-Sheet 2

FIG. 5.



FIG. 6.



FIG. 7.



FIG. 8.



Inventor.

Septimus H. Griffiths

By Jas. L. Skidmore.

Attorney.

## UNITED STATES PATENT OFFICE

2,169,797

METHOD OF CASTING, SELF-STRIPPING AND  
RAPID-COOLING STEEL INGOTS

Septimus H. Griffiths, Canton, Ohio

Application December 31, 1937, Serial No. 182,900

2 Claims. (Cl. 22—212)

This invention pertains to a new and meritorious method of self-stripping an ingot from its mold, and at the same time to eliminate the formation of certain defects frequently known to exist in the cast ingot product, such as "piping," "blow holes" and internal dendritic ruptures well known to those skilled in the art as "internal point cracks."

The prime objects of the invention are to provide a new, simple and improved method of self-stripping the ingot from its mold, said method at the same time serving to eliminate certain defects that are known to exist within the ingot by seating the ingot on its support in spaced relation thereto, maintaining the ingot within the major mold section in spaced relation to the inner wall thereof, permitting cool air to contact and freely circulate within and through the space formed between the peripheral wall of the ingot and the inner wall of said major section, thus subjecting the said walls to a more rapid and uniform cooling thereof, and serving to more thoroughly and completely solidify the ingot, and to materially increase the quality, quantity and value of the ingot product, within a given period such as are made by the use of a big-end-up type of mold, and from any known type of steel, or grades of metal heretofore utilized in connection with this art for the production of ingots.

The disclosure herewith is illustrative of one of the preferred means employed in carrying out the method set forth constituting this invention, and, therefore, is not considered in the limiting sense, since it is evident that this method may be carried out with structures other than those specifically disclosed herewith.

The foregoing and such other objects as may appear from the ensuing description are accomplished by the combination, arrangement, location and construction of the several parts hereinafter more fully described, illustrated in the accompanying drawings, and more particularly pointed out and hereinafter described.

In the accompanying drawings forming a part of this specification, showing one of the preferred types of mold employed in carrying out this invention, it will be seen:

Figure 1 is a side elevation of the type of sectional mold employed in connection with my invention, showing means broken away and attached to the upper section for lifting it away from the lower section.

Figure 2 is a side elevation of the mold, showing means attached to the lower section and to

the mold support for fixedly securing the lower section to said support.

Figure 3 is a sectional elevation of the mold shown in Fig. 1 with the lifting means removed.

Figure 4 is an enlarged sectional view taken in the plane shown by dotted lines 4—4, Fig. 2.

Figure 5 is a side elevation of the large upper section of the mold, showing said section and the lifting means partly in section and partly in full lines with the lower end portion of the ingot seated upon its support.

Figure 6 is a sectional elevation of the large upper mold portion in cross section, the lifting means, ingot, and the ingot support in full lines, and showing the meeting face of the said mold portion disposed in spaced relation with the said support, and the ingot in spaced relation with the inner wall of the mold portion with arrows indicating how the cool, fresh air flows beneath the meeting face of the mold section into contact with the outer wall of the ingot and the inner wall of the major mold section.

Figure 7 is an inverted plan of the upper section of the mold, and

Figure 8 is a plan of the lower section of the mold.

In the embodiment of the mold employed in connection with this invention it will be seen that the numeral 2 designates the major upper section of the mold formed with a laterally extended lug 30 at each side of its upper end portion for the reception of suitable detachable lifting means 4 for lifting and moving the section away from contact with the lower minor section 5 of the mold, lower end of said major section at two opposite sides thereof being provided with a continuous depending extension 6 in alignment with its outer wall and formed at its lowermost end portion with a horizontal seating face 7 and an upwardly and inwardly beveled portion 8 terminating with a vertical wall or shoulder 9 which terminates at the horizontally extended meeting face 10 of the section forming the point of junction with the upper face of the minor section, as is clearly shown in Fig. 3 of the drawings, 45 while the lower minor section 5 is formed at its upper end with similar but upwardly extended integral formations 11 at opposite sides thereof in alignment with its outer wall, and reversely beveled, as shown in Fig. 4, so that when it is 50 desired to join the sections together it is simply necessary to lower the upper section until its lower extended beveled portions contact with the upper and outer end portions of the minor section, when by further lowering said upper sec- 55

tion it will be automatically guided to the point of juncture of the two sections into contact with each other, with the extensions 6 of the major section overlapping the outer wall of the upper end portion of the minor section at opposite sides thereof, and the upward extensions 11 of the minor section overlapping the lower outer walls of the upper section at its opposite sides and above its meeting face, as shown by the dotted lines in Figs. 1 and 2, while the vertical shouldered or wall portions of the extensions 6 and 11 simultaneously serve to embrace and contact with the outer wall of the upper portion of the lower section and the outer wall of the upper section, respectively, thereby maintaining the sections in proper relation to each other, thus causing the meeting faces of the mold sections which are preferably machined, if desired, so as to form a true, accurate and tight juncture of the said meeting faces when joined together for the ingot casting operation.

Both of the mold sections are preferably formed of cast iron, and when united at the point of juncture the inner wall is inclined inwardly from the top to the bottom thereof, terminating with a concaved solid bottom, said formation being provided for the production of "large-end-up" ingots and for eliminating and dispensing with the use of all types of plugs and other expensive well known equipments heretofore utilized for stripping the cast ingots 12 from their molds.

It will be perceived that by this specially designed type of mold all means heretofore employed for securing and locking the mold sections together at their meeting faces are entirely dispensed with, hence neither time nor labor is required for applying or releasing such means, since the larger upper section 2 is simply lowered and is automatically guided by the coaction of all of the aforesaid beveled extensions until the meeting faces of the mold sections truly and smoothly contact and are held in their properly aligned position by the vertically disposed shouldered or wall portions that extend entirely around the mold at the point of juncture of the said sections.

It will be seen that the lower minor section of the mold is provided with an excess of metal at the bottom thereof serving to more rapidly cool and solidify the bottom portion of the ingot, and is formed with a concaved inner lowermost end portion while its outer wall at the bottom portion thereof is provided with an integral projected lug 13 oppositely disposed for the reception of one end portion of an elongated link 14, said link being adapted to be swung over a fixed lateral extension 15, forming a part of the mold support 16 for the reception of the other portion of the metal link, said link and extensions serving to maintain the said minor section of the mold in fixed position with the mold support as the upper major section of the mold containing the ingot is lifted and moved away from the lower minor section to another position and seated upon its support 16.

The several steps employed in my new and improved method may be described as follows:

When the casting operation shall have been completed, and the outer wall and lower end portion of the ingot has been sufficiently solidified, and the thermal contraction of the metal within the mold has taken place to a certain extent, it is simply necessary to attach the lifting means to the projected lugs of the major section and lift it with its contained ingot away from the fixed

minor section with the lower end portion of the ingot depending below the lowermost face of said major section, subsequently lowering and seating the lowermost end of the ingot upon its support 16, then immediately releasing the lifting tension from the major section, thereby permitting said section to immediately and automatically gravitate until its lowermost end portion is also seated on the support 16 with its meeting face 10 in spaced relation with said support, said gravitation of the major mold section simultaneously stripping and forcing the ingot away from the inner wall of the section and projecting the upper end of the ingot beyond the top of the mold section, so that when the lifting means 4 is properly applied or clamped to the said projecting end portion of the ingot said ingot may be readily lifted from the mold section and conveyed to the soaking pit, heating furnace, or other proper destination, thereby facilitating and simplifying the rapid stripping and production of ingots.

It will be seen that, after the major mold section shall have been removed from the minor section and seated upon the support 16 and around the ingot contained within the major section, the last named section will be maintained in spaced relation above its support with the ingot resting in spaced relation with the inner wall of the major section, thus permitting the free circulation of air beneath the meeting face 10 of the mold section at the point marked by the arrows in Fig. 6, and into the space formed between said inner wall of the section and the peripheral wall of the ingot, thereby subjecting the entire wall of the ingot and the inner wall of the mold section to contact with the air while the ingot remains within said mold section, thus serving to more rapidly, uniformly and thoroughly solidify the ingot; to eliminate the formation of piping, blow holes and other defects hereinbefore referred to, and to produce a more valuable and improved product.

It will be readily evident that this invention is adapted for use in connection with all kinds of molten metals used for casting ingots, especially with relation to what is commonly known in the art as rimming or effervescent metal.

It is well understood in the steel manufacturing art that ingot plants and foundries are fully equipped with various types of lifting and conveying means, which may be readily engaged and disengaged from the molds for transferring them from one place to another, as well as all suitable and desirable types of supporting means therefor, hence, since such equipment forms no part of this invention, it has not been deemed necessary to fully illustrate such equipment.

In order to assure the maintenance of the ingot at all times in spaced relation, and away from contact with the inner wall of the major mold section, as shown in Fig. 6 of the drawings, if required, a small wedge member made of asbestos or other suitable material not shown may be placed within the upper end of the mold section between its inner wall and the wall of the ingot for the purpose aforesaid.

Having thus described my invention, what I claim and desire to secure by Letters Patent is:

1. The method of casting and self-stripping an ingot from a mold divided horizontally into a major upper section, and a minor lower section, each section having extensions at its meeting end serving to form an accurate and tight juncture when joined together for casting purposes, con-

sisting in removing the major mold section with its contained ingot projecting below the lowermost end of said section away from the minor mold section, seating the lowermost end of the 5 ingot on a support, releasing the lifting tension from the major mold section, permitting said major section to automatically gravitate until its lowermost end portion is also seated on the support with its meeting face in spaced relation 10 to said support, said gravitation simultaneously forcing the ingot to be stripped away from the inner wall of the major mold section with its top projecting beyond the top of said section and maintaining the ingot within the mold section in 15 spaced relation to the inner wall of said section, permitting the free flow of cool air beneath said meeting face to contact with the wall of the ingot and the inner wall of the major section to rapidly cool and solidify the ingot, removing the ingot 20 from the upper end of the major section, then conveying the ingot to its proper destination.

2. The method of casting, self-stripping and rapidly cooling a steel ingot within a mold divided horizontally into a major upper section and 25 a minor lower section, each section having extensions at its meeting end serving to form an

accurate and tight juncture when joined together for casting purposes, consisting in removing the major section with a portion of its contained ingot disposed below the lowermost end of the said section away from the minor section, seating the lowermost end of the ingot on a support, releasing the lifting tension from the major mold section, thus permitting the major section to automatically gravitate until its lowermost end is seated on said support with its meeting face in 10 spaced relation with the support, said gravitation simultaneously forcing the ingot to be stripped away from the inner wall of the major section and project the upper end of the ingot beyond the upper end of said section, supporting the 15 ingot within the major section in spaced relation with its inner wall, maintaining the ingot within said mold section to simultaneously permit the free circulation of air into and through the mold section in contact with the inner wall of the major section and the entire wall of the ingot until the entire ingot shall have been rapidly and completely cooled and solidified, then lifting the ingot 20 from the top of the mold section and conveying it to its proper destination.

SEPTIMUS H. GRIFFITHS.

5

10

15

20

25